

(No Model.)

E. P. THOMPSON.  
MANUFACTURE OF CARBON FILAMENTS.

No. 401,606.

Patented Apr. 16, 1889.



INVENTOR:

E. P. Thompson  
By his Atty's

Poped Edgecomb

ATTEST:

Charles A. Tracy  
Caroline E. Davidson

# UNITED STATES PATENT OFFICE.

EDWARD P. THOMPSON, OF ELIZABETH, NEW JERSEY.

## MANUFACTURE OF CARBON FILAMENTS.

SPECIFICATION forming part of Letters Patent No. 401,606, dated April 16, 1889.

Application filed February 4, 1887. Serial No. 226,525. (No model.)

*To all whom it may concern:*

Be it known that I, EDWARD P. THOMPSON, a citizen of the United States, residing in Elizabeth, in the county of Union and State 5 of New Jersey, have invented certain new and useful Improvements in the Process of Manufacturing Filaments for Incandescent Electric Lamps, of which the following is a specification.

10 The invention relates to a process of preparing carbonized filaments and treating them while being built up and formed into the required shape.

15 The object of the invention is to produce a filament which shall be durable, have as great a density as practicable, and possess the qualities requisite for satisfactory service.

20 In general terms the invention consists in first washing the carbonized filament with an inert gas while it is incandescent; second, in throwing off the loose particles while it is being so washed by means of a static current or charge; third, in placing the filament under torsional strain, and, if it is desired, at the 25 same time under tension, causing it to break, thus giving a permanent set to its molecules, and afterward building up and forming the filament into the required shape.

30 The invention will be described in connection with the accompanying drawings, in which—

35 Figure 1 shows, in elevation, an apparatus for carrying out the first steps of the invention, together with a convenient system of circuits; and Fig. 2 illustrates the apparatus employed for forming and building up the filament. Fig. 3 shows a modified device for applying torsion to the filament.

40 Referring to Fig. 1, A represents a suitable bell-jar or containing-chamber for receiving a filament, B, which is to be treated. This filament extends through a glass tube, b. The filament is held at its respective ends by two suitable clamps, c' c<sup>2</sup>, and the tube rests in 45 any convenient manner upon the lower stationary clamp, c', terminating above or extending within the gas-supply tube d, extending from any suitable reservoir, D, of hydrogen or inert gas. The clamp c' is connected 50 by a conductor, 1, including a suitable resistance, r', with one pole of a generator or other suitable source of electricity, E. The other

pole is connected by a conductor, 2, with the clamp c<sup>2</sup>. A switch, s, serves to open and close the circuit of the generator through the filament when desired. By placing the filament in circuit and admitting hydrogen through the tube d, the filament B will be washed by the gas, which is caused to pass through the tube in contact with the filament. The filament being heated, the rapidity with which the gas passes through the tube is increased, and thus the filament becomes thoroughly washed. This treatment removes from the filament such loose particles as would otherwise be thrown off or removed from the filament after being placed in the lamp by reason of the long-continued action of the attenuated gas within the globe of the lamp, and thus the blackening of the globe is, to a 7 corresponding extent, prevented. Another advantage resulting from this treatment is that the deposit of carbon, which is subsequently applied, is now made directly upon the solid structural carbon, whereas without such treatment there will necessarily remain upon the filament more or less of the carbon powder or dust in which it is first carbonized, so that the deposited carbon does not have a solid basis and is more easily thrown off. 8c By the present invention, however, the deposited carbon becomes firmly attached to the structural carbon or the real base of the filament.

For the purpose of assisting in the removal 85 of the imperfectly-attached carbon, it is usually preferred to send a static charge of electricity to the filament during the process just described, thus combining with the current by which it is heated to throw off whatever 90 carbon may not otherwise be removed by simply washing. This is conveniently accomplished by connecting the opposite poles of any suitable source of static electricity—such, for instance, as a Leyden jar, F—through the 95 filament. A convenient method of doing this consists in connecting one pole, f, of the jar, which has been previously charged, through a conductor, 3, to the clamp c<sup>2</sup>, and the other pole, f', through a conductor, 4, with the 100 clamp c'. The sudden discharge of the condenser through the filament will produce the required result. In other instances it may be found convenient to use a static generator—

such, for instance, as a Holtz machine or an inductorium. After the filament has been thus treated to the required extent, it is desired to place it under torsion and to cause it to break while it is still heated by the current from the generator E. This current is preferably increased at the proper moment by cutting out any required amount of the resistance  $r'$ . The cutting out of this resistance may serve as a test for determining the strength of the filament to resist fracture under the influence of heat, the amount of current which it is desired that the filament shall stand without injury having been previously determined.

The torsion to which the filament is subjected is also regulated, and it is previously determined how much torsion it shall be capable of withstanding. The torsion is conveniently applied by means of a revolving support,  $h$ , carrying the clamp  $c^2$  and provided with an armature,  $h'$ . An electro-magnet, H, placed outside the chamber A, is applied to this armature, and by turning it in its support it will cause the armature  $h'$ , and thus the support  $h$ , to turn, carrying with it the clamp  $c^2$ , and thus applying torsion to the filament B.

The electro-magnet H may be included in a branch circuit of the generator E, or in any suitable manner placed in an electric circuit. The pointer or indicator  $j$  serves, when the inclosing walls are of transparent material, to indicate upon the plate  $j'$ , carrying the support  $h$ , the amount of torsion thus applied to the filament, and whether or not it withstands the predetermined requisite amount of torsion without breaking. A spring,  $j^3$ , presses against the support  $h$ , and, if it is desired to place the filament under tension while the torsion is applied, the magnet H is vitalized sufficiently to overcome more or less the tension of the spring, thus raising the support  $h$ .

The torsion may be applied to the filament, if desired, before it is placed in the treating jar A, and this may be conveniently accomplished by constructing the clamp  $c^2$  and its support as shown in Fig. 3, in which the support  $h$  carries a handle,  $h^2$ , by means of which it may be conveniently turned above the dial  $j'$ . A series of holes,  $h$ , in the dial-plate receives the pin  $k'$ , carried by the spring-handle  $h^2$ , for holding the support in any required position. Thus the filament may be placed under any predetermined tension and held there during the process of treatment. After the filament has been thus treated, it is desired to break it while it is still under torsion, and for this purpose the increased current already referred to is sent through it, its strength being increased to such a point as will cause it to break. The breaking of the filament while thus subjected to an intense heat will cause a torsional permanent set of the molecules. After the filament has thus been prepared, it is removed from the jar A and treated in a manner which will be de-

scribed in connection with Fig. 2. This consists in first bending the filament into the required shape in any desired or convenient manner and in placing it in suitable supports or clamps,  $n'$  and  $n^2$ . It is then inserted in a jar, N, where it is treated by hydrocarbon gas delivered through a pipe, o, an exhaust-pipe, o', being provided for not allowing the escape of gas from the chamber. The filament is connected in circuit with a generator, E', the amount of current therefrom being regulated by a resistance,  $r^2$ , or in any other convenient manner, and the connections of the circuit being controlled by a switch,  $s'$ . The filament is thus built up by a deposit of hydrocarbon while it is held in the proper required shape. The gas applied to the filament in this manner is preferably under greater or less pressure, the amount of which may be readily determined by means of a suitable gage, P, applied to the chamber M in any convenient manner. It is not always necessary to apply the carbon deposit in the manner just described; but the hydrocarbon gas may be applied to the filament while it is in the chamber A. (Shown in Fig. 1.) Thus it may, for instance, be supplied through the tube d, a hydrogen-reservoir being disconnected.

It is not desired to confine the individual methods of treating the filament to this entire process; but certain of the steps may be performed without the sequence of the others, if so desired. In some instances it is desired to reduce the size of the filament by removing more or less of the outer surface, and the torsional treatment may be employed without breaking the filament during the process of washing or removing the partially-detached particles. The torsion which is put into the filament will cause the outer fibers to break, and these may be removed in the manner already described, thus reducing the cross-section of the filament.

The chamber A is preferably composed of some suitable refractory substance—such, for instance, as fire-clay—for the purpose of confining the heat, and this is surrounded by a glass tube A', which assists in preventing the access of air into the chamber by having the end upon which it rests ground to fit tightly to the support or base. Between these two walls, therefore, there will be a space occupied by a more or less attenuated gas.

The treatment of the filament by twisting and heating by the current may be alternated, if desired, the required amount of torsion thus being gradually applied.

The filament may be broken by twisting it alone without increasing the strength of current, and a sufficient permanent set may be obtained in some instances in this manner.

I claim as my invention—

1. The hereinbefore-described process of treating filaments, which consists in washing the same by a current of inert gas, heating the filament while being so washed, and in

sending a static charge to said filament while being so washed.

2. The hereinbefore-described process of treating filaments, which consists in removing the loose particles of carbon from the filament by a static charge of electricity and in building up the filament by a deposit of carbon upon the filament, substantially as described.

10 3. The hereinbefore-described process of treating filaments, which consists in washing the filament by an inert gas, heating the filament to incandescence while being so washed, throwing off the loose particles by one or more 15 static charges, and in subsequently building up the filament by a deposit of carbon.

4. The hereinbefore-described process of treating filaments, which consists in washing them with gas while incandescent, subsequently placing them under torsion, and breaking them while under torsion.

5. The hereinbefore-described process of treating filaments, which consists in washing them with gas while incandescent, subsequently placing them under torsion, and in

heating them by an increased current until they break.

6. In an apparatus for treating filaments for incandescent electric lamps, the combination, with an inclosing-case, of clamps for supporting the filament, a revolving support for one of the clamps, an armature carried thereby, and an electro-magnet outside of said case for revolving the armature.

35 7. In an apparatus for treating filaments for incandescent electric lamps, the combination, with an inclosing-case, of clamps for supporting the filament, a revolving support for one of the clamps, an armature carried thereby, an electro-magnet outside of said case for 40 revolving the armature, and a spring acting in opposition to the longitudinal pull of said electro-magnet.

In testimony whereof I have hereunto subscribed my name this 21st day of January, A. 45 D. 1887.

EDWARD P. THOMPSON.

Witnesses:

DANL. W. EDGEcomb,  
CHARLES A. TERRY.